

April 20, 1937.

L. G. DAY

2,077,990

MELTING, REFINING AND PREPARATION FOR CASTING OF MAGNESIUM AND LIKE METALS

Filed May 29, 1936

2 Sheets-Sheet 1



*L. G. Day  
inventor*

*By: Glascock, Downing & Sebold  
Attns.*

April 20, 1937.

L. G. DAY

2,077,990

MELTING, REFINING AND PREPARATION FOR CASTING OF MAGNESIUM AND LIKE METALS

Filed May 29, 1936

2 Sheets-Sheet 2

Fig.2



L. G. Day  
inventor

By: *Mascot Downing, Seebold*  
Atty.

## UNITED STATES PATENT OFFICE

2,077,990

MELTING, REFINING AND PREPARATION  
FOR CASTING OF MAGNESIUM AND  
LIKE METALS

Leslie George Day, Taplow, England, assignor to  
Magnesium Castings and Products Limited,  
Slough, England and to High Duty Alloys  
Limited, Slough, England

Application May 29, 1936, Serial No. 82,644  
In Great Britain June 7, 1935

9 Claims. (Cl. 75—65)

The present invention relates to the melting, refining and preparation for casting of metals such as magnesium or magnesium alloys which in the molten form are subject to attack in the presence of the air. The invention relates in particular to operations of the kind in which a stock of the molten metal is provided in a pot or furnace and portions of the stock are withdrawn from time to time for casting.

It is generally known that great difficulties are encountered in melting and casting magnesium and its alloys owing to the great affinity which the metal has for oxygen and nitrogen. This affinity is such as to make an open bath of the metal unworkable unless the surface is covered with a layer of protective flux. The use of such a flux has several serious disadvantages, the chief of which is that particular care must be exercised in pouring or otherwise removing the metal from beneath the flux without entraining the flux with the molten metal, and even with meticulous care there is a likelihood of a certain proportion of flux being entrained.

It has been proposed to use inert gases for protecting the surface of the molten metal, but when working with a stock of such metal from which portions are withdrawn with the aid of a ladle eddying of the gases occurs at the aperture through which the ladle is inserted and consequently air enters the furnace and attacks the surface of the metal. Moreover, the inert gases which may be used, for example sulphur dioxide, are usually of such nature that any substantial concentration thereof is injurious to the operatives and consequently it is not feasible to prevent the entry of air into the furnace by supplying a rapid stream of the inert gas to within the furnace, or completely effective use of an inert gas in a totally enclosed container might be used in certain circumstances, but it is obviously impracticable in melting and ladling operations of the kind described.

The present invention consists in a method of melting, refining and preparing for casting of metal such as magnesium in a furnace having an aperture above the surface of the metal of size sufficient to admit a ladle, according to which an inert gas is slowly introduced into or generated within the furnace, either continuously or intermittently, above the surface of the metal and a gas flow is established adjacent to the aperture and in a plane substantially parallel to the plane of the said aperture, the extent and the velocity of the gas flow being sufficient to prevent the entrance of air through the aperture.

In carrying out the present invention it is preferred to establish the gas flow by means of a number of jets of combustible gas, e. g. ordinary coal gas, which burn and are suitably directed in the neighbourhood of the aperture. When establishing the gas flow of this nature it is furthermore preferred to conduct the whole operation under a suitable hood so that the hot products of combustion may be withdrawn to a stack. The draught thus induced facilitates the establishment of a satisfactory gas flow. The combustible gas may for example be supplied from two series of jets located laterally of the aperture and directed inwardly and from another series of jets located beneath the aperture and directed upwardly, the jets in both series lying in a plane parallel to the plane of the aperture. The stream of hot combustion gas thus generated not only serves to prevent any currents of air from entering the furnace, but also serves to carry off the slow stream of inert gas which is supplied within the furnace and which leaks outwardly through the aperture. Thus, when the whole operation is conducted under a suitable hood and the hot products of combustion withdrawn to a stack it is possible to use as the inert gas supplied within the furnace a relatively noxious gas such as sulphur dioxide without harmful effect on the operatives. Other inert gases may be admitted, however, within the furnace such for example as carbon monoxide, carbon dioxide or the products of combustion for example of ordinary coal gas.

One way of carrying the invention into effect will now be described with reference to the accompanying diagrammatic drawings, wherein:—

Figure 1 represents a front elevation of a furnace, and

Figure 2 is a sectional elevation through the centre of Figure 1.

Referring to the drawings:—

A circular oil or gas-fired melting furnace 1 contains a suitably-shaped melting pot 2 covered by a dome-shaped cover 3 which is jointed by flanges and an asbestos ring 4 to the pot 2.

A vertical aperture 5 of a size which will permit of the introduction of the ladle is formed in the cover 3, which latter is also provided with several small holes 6 through which a supply of sulphur dioxide may be introduced into the space 7 above the molten metal 8 by way of the pipe 9. The positioning of these inlet holes 6 should be such that the inert gases let in above the metal should come in at as many points as possible and

be so distributed that the gas readily covers the whole surface of the metal.

In the particular example under consideration two of these inlet holes are placed close to the aperture. A gas burner in the form of two vertical arms 10, 11 rising from a horizontal portion 12 is placed immediately in front of the ladling aperture 5 so as to frame the aperture on three sides.

10 The plane of the burner is substantially parallel to the plane of the mouth of the ladling aperture and the three parts of the burner are perforated along their inner sides in such a manner as to tend to throw jets of burning gas across the 15 aperture in the plane of the burner. Situated vertically above the burner and aperture is a hood 13 and stack pipe 14 arranged in such a manner that the hot gases from the burner together with excess protective gases are collected 20 by the hood and forced up the stack pipe.

Sliding doors 15, 16 normally close the aperture 5 but are moved aside when a ladle is to be introduced for the removal of metal for casting.

In carrying out the melting operation in the 25 above described apparatus, the crucible 2 is charged with a suitable quantity of magnesium and heavy density flux.

As soon as the melting commences the part of 30 the pot above the molten metal is filled with sulphur dioxide and the gas ignited on the burner 10, 11, 12 in front of the aperture. A slow stream of sulphur dioxide into the pot is then maintained during the whole of the succeeding operations. The metal when molten is stirred up with 35 the flux which sinks to the bottom and the metal may then be raised to temperatures considerably above those usual in casting without the slightest trace of the burning or sparking which is usual on the surface of molten magnesium. The 40 gas burner, hood and stack pipe prevent air from being carried on to the surface of the molten magnesium and at the same time leaves the metal freely accessible for stirring, skimming, ladling or other operations connected with its operation for 45 casting.

#### General

Inert gases other than sulphur dioxide, for instance, carbon dioxide, carbon monoxide, or the rare gases argon, helium, neon, krypton, xenon 50 may be used for filling the space above the molten metal and means other than the gas jets described above may be used for producing the desired sealing gas stream.

The process described above is of particular 55 advantage in those cases where a large charge of metal is kept at the optimum temperature for casting and has to be distributed among a number of moulds, since by this process each casting may be made with metal of the same temperature.

60 The aperture should be of such size as to permit of the free use of a suitable ladle and may therefore be utilized for inspection or manipulation of the charge for example stirring under visual control, or for charging and recharging the 65 furnace during the melting operation.

Having now described my invention, what I claim as new and desire to secure by Letters Patent is:—

1. A process for the melting, refining and preparation for casting of light metals such as 5 magnesium or magnesium alloys, which are vigorously attacked by air when molten, which consists in melting the metal in a covered crucible having an aperture above the surface of the metal in a substantially vertical plane and of a size sufficient to admit a casting ladle, maintaining an atmosphere of inert gas above the surface of the metal at a pressure slightly above that of the atmosphere and passing an independent sealing gas stream adjacent to and substantially parallel 10 to the plane of the face of the said aperture on the outer side thereof.

2. A process as claimed in claim 1 wherein the inert gas atmosphere is maintained by slowly passing inert gas into the space above the surface of 20 the metal.

3. A process as claimed in claim 1 wherein the inert gas atmosphere is maintained by generating inert gas in the space above the surface of the metal.

25 4. A process as claimed in claim 1 wherein the gas stream consists of hot combustion gases.

5. A process as claimed in claim 1 wherein the gas stream consists of hot combustion gases generated by a series of jets of combustible gases arranged partially around the aperture.

30 6. A process as claimed in claim 1 wherein the gas stream consists of hot combustion gases which are drawn off by a suitable hood and stack arranged above the aperture.

35 7. A process as claimed in claim 1 wherein the inert gas is sulphur dioxide.

8. Apparatus for melting, refining and preparing for casting metals such as magnesium including a covered crucible having an aperture of 40 considerable size and in a substantially vertical plane above the molten metal level, means for covering the molten metal with an inert gas at a pressure slightly above that of the atmosphere and means for producing an independent stream 45 of gas adjacent to and across the aperture so as to prevent the passage of atmospheric air therethrough.

9. Apparatus as claimed in claim 8 wherein the aperture in the upper part of the crucible is normally closed by suitable doors, the means for covering the surface of the metal with inert gas comprises a series of inwardly directed nozzles arranged around the circumference of the crucible and the means for producing the stream of gas 50 comprises a burner arranged close to and around the sides and bottom of the aperture so as to project jets of burning gas in a plane close to and substantially parallel to the plane of the orifice and a hood and stack pipe arranged above the 55 burner to carry off the products of combustion and any excess inert gas from the interior of the crucible.

LESLIE GEORGE DAY.

65